

# UNITED STATES PATENT OFFICE.

FREDERICK P. WOOD, OF OAK PARK, ILLINOIS, ASSIGNOR TO AMERICAN CAN COMPANY, OF NEW YORK, N. Y., A CORPORATION OF NEW JERSEY.

## PROCESS OF PROOFING MATERIALS.

1,310,818.

Specification of Letters Patent. Patented July 22, 1919.

No Drawing.

Application filed May 28, 1915. Serial No. 30,911.

To all whom it may concern:

Be it known that I, FREDERICK P. Wood, a subject of the King of Great Britain, residing in Oak Park, in the county of Cook 5 and State of Illinois, have invented a new and useful Improvement in Processes of Proofing Materials, of which the following is a specification.

This invention relates in general to the 10 proofing of paper or fibrous materials and has more particular reference to the proofing of such articles in order that they may be used for the containing of fats, oils and the like.

15 My present invention has reference to the forming of a can or container body of the type and characteristics described in my pending application for containers filed March 5, 1915, Serial No. 12306.

20 In providing a paper or fibrous container adapted for the packaging of lard, lard substitutes and other greases and the like, I have found it advisable to coat the bodies of such containers with an infusible substance 25 insoluble in the intended contents of the containers when in their most fluid condition. This proofing substance, to attain the best results, should be applied in the form of a continuous film over the body of 30 the container. This invention has for its principal object the provision of a process or method for the forming of such a film.

35 A further object of the invention is the provision of a method or process for coating articles of the character and in the manner described, which may be easily practised commercially and which will insure the production of containers of high and uniform quality.

40 Other objects and advantages of the invention will be apparent as it is more fully understood from the following description which is of a specific embodiment of it.

The coating may have varying characteristics and be formed of materials of different qualities without departing from the spirit of the invention. I have found however in using a coating of the character described in my pending application, to 45 which reference has already been made, that if the material of the coating be permitted to penetrate the body of the container, considerable difficulty is experienced in the

formation of the continuous film desired and this by reason of the fact that the 55 capillary action, which is present when the coating material is of sufficiently low viscosity, causes the absorption of the film, which absorption however is not sufficient to prevent subsequent seeping out of the 60 contents, the result of this absorption being merely a coating of the fibers of the container body as contradistinguished from a coating of the surface.

In accordance with my invention it is 65 intended to control the fluidity of the bath in which the container bodies are immersed for coating at such a viscosity that this permeation will be reduced at least sufficiently to insure the formation of a coating upon 70 the surfaces desired to be protected.

This control of the fluidity I accomplish in the present instance by a control of the temperature of the bath in which the cans are immersed for coating. If hide glue be 75 used as a proofing substance this temperature should be in the neighborhood of 110° F., for I have found that at or about that temperature it is best adapted to produce a surface film upon paper or other porous 80 material. At that temperature also its adhesive qualities are well developed and it is not so viscous as to form a coating of undesirable thickness.

It will be manifest that other means than 85 that of heat control may be provided for regulating the viscosity or fluidity without departing from the spirit and scope of the invention, it only being necessary that this viscosity be so controlled as to form the film 90 without appreciable permeation or saturation of the body receiving it. After the coating has been applied the containers are removed from the bath and the coating set by drying at like or lower temperatures in 95 order that the film produced in the bath may not be destroyed.

It is thought that the invention and many 100 of its attendant advantages will be understood from the foregoing without further description, and it will be obvious that various changes may be made in the steps of the process described and in the materials operated with and upon without departing from the spirit and scope of the invention or 105 sacrificing any of its material advantages,

the process hereinbefore described being merely a present preferred embodiment thereof.

I claim:

- 5 1. The process of proofing paper container bodies, which consists in providing a suitable grease repelling coating material in fluid and viscous state, said coating being capable of being hardened by drying, maintaining by heat the fluidity of said coating at a viscosity which will restrain absorption by the capillary action of the material of the body of said container, applying said coating directly on the surface only of a 15 fibrous container body and hardening the coating thus formed on said container body whereby said coating is in the form of a continuous surface film.
- 20 2. The process of proofing fibrous container bodies which consists in immersing a container in a grease-repelling coating material capable of variable viscosity at different temperatures, and maintained at a temperature which will give only sufficient 25 viscosity to coat the surface of said con-

tainer but restraining the permeating of the container by capillary action, and subsequently drying and hardening said coating.

3. The process of proofing paper container bodies which consists in applying 30 hide glue to fibrous container bodies at a viscosity and degree of heat which will restrain permeation into said bodies, and subsequently drying and hardening said coating under conditions preventing increased 35 fluidity.

4. The process of proofing container bodies which consists in applying hide glue directly to a fibrous container body under a temperature of about 110°F. which will 40 maintain the coating in a sufficiently viscous state to restrain permeation of the body, and subsequently drying at like or lower temperature.

Signed in the presence of two subscribing 45 witnesses.

FREDERICK P. WOOD.

Witnesses:

J. C. CARPENTER,  
ESTHER ABRAMS.